

**3,282,731**  
**EMBRITTLEMENT-FREE PICKLING OF**  
**FERROUS METAL**

Robert M. Hudson, Churchill Borough, and Kermit J. Riedy, King of Prussia, Pa., assignors to United States Steel Corporation, a corporation of Delaware  
No Drawing. Filed May 28, 1963, Ser. No. 283,717  
6 Claims. (Cl. 134—41)

This invention relates to limiting the hazards of hydrogen embrittlement and overpickling during removal of oxide scale from ferrous metal by acids. 10

Iron and steel products become coated with an oxide scale during their process of manufacture, the presence of which is objectionable in their further processing, as for example in coating the products or forming them by drawing in dies. A conventional method of scale removal involves contacting the material with an aqueous solution of an inorganic acid, typically sulfuric acid, usually by immersion in a bath thereof. Since the acids employed are capable of dissolving the base metal, a reaction which is more rapid than that of oxide dissolution, pitting of the metal results where acid attacks it through discontinuities in the oxide film. Also, after the oxide layer has been removed, continued contact of the metal with the acid results in undesirable dissolution of metal, a condition known as overpickling. Moreover, hydrogen produced in the metal dissolution reaction increases the likelihood of hydrogen embrittlement of the ferrous base, which latter condition results from absorption of hydrogen by the base metal. 30

In order to alleviate the foregoing difficulties, it is common practice to add to the pickling solution an inhibitor for the metal dissolution reaction, thus permitting more selective action in effecting oxide removal and reducing hydrogen production. 35

It has been noted that the degree of prevention of hydrogen embrittlement during pickling, resulting with various inhibitors, is unpredictable, some inhibitors even increasing embrittlement.

The present invention concerns inhibited acid pickling solutions capable of controlling acid attack of the base metal, which solutions contain inhibitors which are markedly effective as well in preventing hydrogen absorption, with its resulting embrittlement effect. These results are obtained by the addition, to the pickling acid solutions, of an acetylenic carboxylic acid, which may be acetylene dicarboxylic acid or propiolic acid.

We have found that acetylene dicarboxylic acid is effective when used in the concentration range of 11 to 91 grams per liter of a 2 N sulfuric-acid solution and that propiolic acid is effective when used in the concentration range of 3.5 to 28 grams per liter of a similar acid solution. 50

Additional data, as to approximate useful ranges of inhibitor concentration, are presented in Table I.

TABLE I.—GRAMS INHIBITOR PER GRAM EQUIVALENT WEIGHT OF PICKLING ACID

|                                  | Effective Range, g. | Preferred Range, g. |
|----------------------------------|---------------------|---------------------|
| Acetylene dicarboxylic acid..... | 4 to 70             | 5 to 45             |
| Propiolic acid.....              | 1 to 28             | 2 to 15             |

Table II is illustrative of test results obtained with the new pickling inhibitors. A commercially normalized and temper-rolled low-carbon sheet steel having the following composition was used: 0.022% C, 0.09% Mn, 0.009% P, 0.046% S, 0.006% Si, 0.01% Cu, 0.01% Ni, 0.01% Cr, 0.007% Al, the balance being essentially iron. The steel thickness was .035 inch and coupons of 2 by  $\frac{3}{8}$  inch were

cut and vapor degreased with trichloroethylene before use. The specimens were pickled at 100° F. for various selected times up to 24 hours by immersion in either uninhibited 2 N sulfuric-acid solutions or 2 N sulfuric-acid solutions containing various concentrations of inhibitors. 5 Specimens were weighed prior to pickling and after extraction of the hydrogen absorbed during pickling. The hydrogen concentration in pickled steel was determined by warm extraction at 160° C., according to the method described by R. M. Hudson, J. K. Magor, and G. L. Stragand (J. Amer. Ceram. Soc. 41, 23 (1958)).

TABLE II.—METAL DISSOLUTION AND HYDROGEN PICK-UP IN 2 NORMAL SULFURIC-ACID SOLUTION AT 100 F.

| Inhibitor                        | Inhibitor Conc., g./l. | Weight Loss, mg./cm. <sup>2</sup> |        | Hydrogen Absorbed, cc./100g. |        |
|----------------------------------|------------------------|-----------------------------------|--------|------------------------------|--------|
|                                  |                        | 4 hr.                             | 24 hr. | 4 hr.                        | 24 hr. |
| None.....                        | 0                      | 21.1                              | 130.2  | 8.3                          | 19.1   |
|                                  | 5.7                    | 11.4                              | 75.5   | 3.1                          | 10.1   |
|                                  | 11.4                   | 2.1                               | 19.5   | 1.5                          | 2.9    |
| Acetylene dicarboxylic acid..... | 22.8                   | 3.8                               | 28.6   | 0.7                          | 1.1    |
|                                  | 45.6                   | 3.4                               | 10.4   | 0.9                          | 0.8    |
|                                  | 91.2                   | 2.7                               | 13.0   | 0.7                          | 0.6    |
|                                  | 138.8                  | 2.1                               | 26.0   | 1.7                          | 4.2    |
|                                  | 0.7                    | 5.3                               | 59.9   | 5.6                          | 8.6    |
|                                  | 3.5                    | 1.7                               | 3.9    | 1.6                          | 1.7    |
| Propiolic acid.....              | 14.0                   | 0.6                               | 2.6    | 0.7                          | 1.1    |
|                                  | 28.0                   | 3.0                               | 6.5    | 1.0                          | 1.1    |
|                                  | 56.0                   | 6.1                               | 18.2   | 1.7                          | 1.3    |

It will be appreciated that the foregoing concentration ranges and specific examples are illustrative only, to permit ready practice of the invention, and that such variations in concentrations and combinations of ingredients as would occur to those familiar with the art to which this invention appertains are included herein and are within the scope of the following claims.

We claim:

1. A method for embrittlement-free pickling of ferrous metal comprising the step of subjecting said metal to an aqueous solution consisting essentially of a strong mineral acid, adapted to pickle ferrous metal, and an acetylenic carboxylic acid selected from a group consisting of acetylene dicarboxylic acid and propiolic acid, the concentration of said latter acid being sufficient to inhibit dissolution of the ferrous metal and to reduce hydrogen absorption therein.
2. The method of claim 1 in which said pickling acid is sulfuric acid.
3. A method for embrittlement-free pickling of ferrous metal comprising the step of subjecting said metal to an aqueous solution consisting essentially of a strong mineral acid, adapted to pickle ferrous metal, and acetylene dicarboxylic acid, concentration of said latter acid being sufficient to inhibit dissolution of the ferrous metal and to reduce hydrogen absorption therein.
4. A method for embrittlement-free pickling of ferrous metal comprising the step of subjecting said metal to an aqueous solution consisting essentially of a strong mineral acid, adapted to pickle ferrous metal, and propiolic acid, the concentration of said latter acid being sufficient to inhibit dissolution of the ferrous metal and to reduce hydrogen absorption therein.
5. A method for embrittlement-free pickling of ferrous metal comprising the step of subjecting said metal to an aqueous solution consisting essentially of a strong mineral acid, adapted to pickle ferrous metal, and acetylene dicarboxylic acid, said latter acid being present in concentration range of about 5 to 45 grams per gram equivalent weight of pickling acid.
6. A method for embrittlement-free pickling of ferrous metal comprising the step of subjecting said metal to an

aqueous solution consisting essentially of a strong mineral acid, adapted to pickle ferrous metal, and propionic acid, said latter acid being present in concentration range of about 2 to 15 grams per gram equivalent weight of pickling acid.

5

2,993,864 7/1961 Monroe et al. 252—146 X  
3,049,496 8/1962 Monroe et al. 252—146  
3,114,657 12/1963 Stilwell 252—79.4  
468,231 3/1943 Italy.

## FOREIGN PATENTS

## References Cited by the Examiner

## OTHER REFERENCES

## UNITED STATES PATENTS

Raphael, Acetylenic Compounds in Organic Synthesis, Academic Press Inc., pub. New York, 1955, pp. 81 and 82.

2,344,404 3/1944 Giloy 252—146 X  
2,899,391 8/1959 Mayhew et al. 106—14 10  
2,993,862 7/1961 Monroe et al. 252—146  
2,993,863 7/1961 Monroe et al. 252—146 X

JOHN H. MACK, Primary Examiner.  
R. MIHALEK, Assistant Examiner.